

3,329,477

## METHOD FOR PRINTING DYESTUFFS AND PRINTING PASTES

David F. Mason and Thomas E. Lesslie, Mount Holly, N.C., assignors to Martin-Marietta Corporation, a corporation of Maryland  
 No Drawing. Filed Mar. 11, 1963, Ser. No. 264,044  
 6 Claims. (Cl. 8—70)

The present invention relates to a method for printing dyestuffs on textile fibers, and more particularly to a method for printing dyestuffs selected from the group consisting of sulfur dye, azo-disulfide dyestuff, and mixture of sulfur dye and azo-disulfide dyestuff on textile fibers, and to printing pastes useful therein.

The method of the present invention is particularly characterized in that a delayed action reducing agent selected from the group consisting of



wherein  $\text{R}_1$  and  $\text{R}_2$  are alkylene groups having 1-5 carbon atoms, a salt of said



and sodium S-sodiocarboxymethyl thiosulphate is used as a delayed action reducing agent for the dyes, providing surprising advantages which will be hereinafter described. The method of the present invention is further characterized in that it comprises the steps of applying to the textile fibers a printing paste comprising water, thickening agent, alkali, a reducing agent selected from the group consisting of



wherein  $\text{R}_1$  and  $\text{R}_2$  are alkylene groups having 1-5 carbon atoms, a salt of said



and sodium S-sodiocarboxymethyl thiosulphate, and dyestuff selected from the group consisting of sulfur dye, azo-disulfide dyestuff, and mixture of sulfur dye and azo-disulfide dyestuff; steaming the fibers to activate the reducing agent and reduce the dyestuff; and oxidizing the dyestuff. If desired, a solubilizing agent and hydroscopic agent may be advantageously included in the printing paste.

The printing paste of the present invention comprises water, thickening agent, alkali, a reducing agent selected from the group consisting of



wherein  $\text{R}_1$  and  $\text{R}_2$  are alkylene groups having 1-5 carbon atoms, a salt of said



sodium S-sodiocarboxymethyl thiosulphate, dye selected from the group consisting of sulfur dye, azo-disulfide dyestuff and mixture of sulfur dye and azo-disulfide dyestuff, and optionally a solubilizing agent and hydroscopic agent.

Until recent years, there was very little printing of sulfur dyes because corrosion of printing rollers resulted, particularly expensive engraved chromium plated copper printing rollers.

Although a number of prior proposals have been made to eliminate the problem of roller corrosion in connection with printing sulfur dyes, the only two proposals which

were used commercially were methods wherein either glucose-carbonate or sodium formaldehyde hydrosulphite were used as the reducing agent for the sulfur dye. However, these two methods have the disadvantage of giving poor color yield with some of the sulfur dyes, and the additional disadvantage of failure to develop the brightest shade of a number of sulfur dyes.

Azo-disulfide dyestuffs have been known for more than fifty years, but have not gone into commercial production or use, one of the principal reasons being that a commercially acceptable method for dyeing and printing the azo-disulfide dyestuffs has remained unknown. Insofar as can be determined, no one has previously suggested a method for printing azo-disulfide dyes.

Moreover, no one has suggested a method for printing a mixture of sulfur dye and azo-disulfide dyestuff.

The term azo-disulfide dyestuff as used herein may be defined as the group of dyes having a reducible disulfide group ( $-\text{S}-\text{S}-$ ) connected between aromatic nuclei to which are attached color bodies containing azo groups ( $-\text{N}=\text{N}-$ ), and also the group of dyestuffs which, upon reduction and oxidation, produce a disulfide group connected between aromatic nuclei to which are attached color bodies containing azo groups. The azo groups may either be connected to the same aromatic nuclei to which the disulfide group is connected, or they may be found elsewhere in the color bodies. Illustrative examples of the above three types of azo-disulfide dyestuffs are the dyestuff formed by coupling one mole of diazotized 5-thiocyanato-2-amino-toluene to one mole of beta-naphthol, which dyestuff upon reduction and subsequent oxidation produces 3:3'-dimethyldiphenyldisulfide 4:4'-bis-(azo-beta-naphthol); the dyestuff formed by coupling one mole of diazotized para-nitroaniline to one mole of 1-phenyl-3-methyl-5-pyrazolone, reducing and diazotizing the resulting product and coupling it to one-half mole of beta-hydroxynaphthoic acid dithioanilide; and the dyestuff formed by coupling one mole of tetrazotized 4:4'-diaminodiphenyldisulfide to two moles of 1-phenyl-3-methyl-5-pyrazolone.

Although sodium sulphide has been suggested as a reducing agent for dyeing azo-disulfide dyes, it is unsuitable for printing azo-disulfide dyes because it corrodes the printing rollers. Also, neither glucose-carbonate nor sodium formaldehyde hydrosulphite may be used as the reducing agent in printing azo-disulfide dyestuffs, or mixtures of sulfur dye and azo-disulfide dyestuff.

According to the method and printing paste of the present invention, the above disadvantages and limitations of the prior art have been overcome, and additional advantages have been provided as follows.

It has been found that sulfur dye, azo-disulfide dyestuff and mixture of sulfur dye and azo-disulfide dyestuff may be printed on cellulosic textile fibers without corroding the engraved printing rollers by the method and with the printing paste of the present invention. Additionally, the method provides improved color yield and improved brightness of shade for some of the sulfur dyes.

The above reducing agents utilized in the present invention are of delayed action type in the sense that they do not reduce the dyestuff until it is in the steamer. The printing paste is applied to the fibers by means of the printing rollers and the printing rollers are not attacked by any of the components in the printing paste. The reduction of the dyestuff occurs in the steamer, as evidenced by the fact that those azo-disulfide dyestuffs and sulfur dyes which have a characteristic color change on being converted to the reduced state undergo this color change in the steamer. The delayed action reducing agent is converted into its active reducing components in the steamer, and corrosion of the printing rollers

is thus avoided. It is believed that all of the delayed action reducing agents break down in the steamer into thioglycollic acid salts or a higher homologue thereof, which are the active reducing agents. For example, if a mole of di(sodiocarboxymethyl) trithiocarbonate,



which does not attack the printing rollers, is used as the delayed action reducing agent and NaOH is used as the alkali in the printing paste, two moles of



(disodium salt of thioglycollic acid) and one mole of



(disodium thiocarbonate) are formed in the steamer by decomposition under heat, but not until a temperature of about 130° F. has been reached.

Several specific and non-limiting examples of the delayed action reducing agents suitable for use in the present invention and having the formulas



wherein  $\text{R}_1$  and  $\text{R}_2$  are alkylene groups having 1-5 carbon atoms, which may be generally referred to as di(carboxyalkyl) trithiocarbonates, are:



The above di(carboxyalkyl) trithiocarbonates may be prepared by reacting disodium trithiocarbonate with a substituted alkyl halide.

Several specific and non-limiting examples of the salts of



wherein  $\text{R}_1$  and  $\text{R}_2$  are alkylene groups having 1-5 carbon atoms, which may be generally referred to as salts of di(carboxyalkyl) trithiocarbonates, and are suitable for use in the present invention are:

- 5       $\text{NaO}-\overset{\text{O}}{\text{C}}-\text{CH}_2-\overset{\text{S}}{\text{C}}-\text{S}-\text{CH}_2-\overset{\text{O}}{\text{C}}-\text{O}-\text{Na}$   
       di(sodiocarboxymethyl) trithiocarbonate
- 10      $\text{NaO}-\overset{\text{O}}{\text{C}}-\text{CH}_2-\text{CH}_2-\overset{\text{S}}{\text{C}}-\text{S}-\text{CH}_2-\text{CH}_2-\overset{\text{O}}{\text{C}}-\text{O}-\text{Na}$   
       di(sodiocarboxyethyl) trithiocarbonate
- 15      $\text{NaO}-\overset{\text{O}}{\text{C}}-\text{CH}_2-\text{CH}_2-\text{CH}_2-\overset{\text{S}}{\text{C}}-\text{S}-\text{CH}_2-\text{CH}_2-\text{CH}_2-\overset{\text{O}}{\text{C}}-\text{O}-\text{Na}$   
       di(sodiocarboxypropyl) trithiocarbonate
- 20      $\text{NaO}-\overset{\text{O}}{\text{C}}-\text{CH}_2-\text{CH}_2-\text{CH}_2-\text{CH}_2-\overset{\text{S}}{\text{C}}-\text{S}-\text{CH}_2-\text{CH}_2-\text{CH}_2-\overset{\text{O}}{\text{C}}-\text{O}-\text{Na}$   
       di(sodiocarboxybutyl) trithiocarbonate
- 25      $\text{NaO}-\overset{\text{O}}{\text{C}}-\text{CH}_2-\text{CH}_2-\text{CH}_2-\text{CH}_2-\text{CH}_2-\overset{\text{S}}{\text{C}}-\text{S}-\text{CH}_2-\text{CH}_2-\text{CH}_2-\text{CH}_2-\overset{\text{O}}{\text{C}}-\text{O}-\text{Na}$   
       di(sodiocarboxyamyl) trithiocarbonate
- 30      $\text{NaO}-\overset{\text{O}}{\text{C}}-\text{CH}_2-\overset{\text{O}}{\text{C}}-\text{CH}_2-\overset{\text{S}}{\text{C}}-\text{S}-\text{CH}_2-\overset{\text{O}}{\text{C}}-\text{CH}_2-\overset{\text{O}}{\text{C}}-\text{O}-\text{Na}$   
       di(1,2-disodiocarboxyethyl) trithiocarbonate
- 35      $\text{NaO}-\overset{\text{O}}{\text{C}}-\text{CH}_2-\overset{\text{CH}_3}{\text{CH}_2}-\text{CH}_2-\overset{\text{CH}_3}{\text{CH}_2}-\overset{\text{S}}{\text{C}}-\text{S}-\text{CH}_2-\overset{\text{CH}_3}{\text{CH}_2}-\text{CH}_2-\overset{\text{CH}_3}{\text{CH}_2}-\overset{\text{O}}{\text{C}}-\text{O}-\text{Na}$   
       di(sodiocarboxyisoamyl) trithiocarbonate
- 40      $\text{NaO}-\overset{\text{O}}{\text{C}}-\text{CH}_2-\overset{\text{CH}_3}{\text{C}}-\text{CH}_2-\overset{\text{CH}_3}{\text{CH}_2}-\overset{\text{S}}{\text{C}}-\text{S}-\text{CH}_2-\overset{\text{CH}_3}{\text{C}}-\text{CH}_2-\overset{\text{CH}_3}{\text{CH}_2}-\overset{\text{O}}{\text{C}}-\text{O}-\text{Na}$   
       di(sodiocarboxytertiaryamyl) trithiocarbonate
- 45     The above salts may be prepared by reacting di(carboxyalkyl) trithiocarbonates with alkali. It will be recognized that other cations may be substituted for sodium in the above trithiocarbonates; however, sodium is preferred for reasons of economy. The salts of the di(carboxyalkyl) trithiocarbonates are preferably formed in the
- 50     55    printing paste when alkali is added to di(carboxyalkyl) trithiocarbonates, and subsequently break down into the active reducing agents under the influence of steam. However, these salts may be prepared prior to their being incorporated into the printing paste.
- 55     60    Sodium S-sodiocarboxymethyl thiosulphate is the sodium salt of S-carboxymethyl thiosulfuric acid, and may be prepared by reacting sodium chloroacetate with sodium thiosulphate.
- 60     65    The reducing agent, while in the steamer, reduces the sulfur dye at its normal reducible site, and reduces azo-disulfide dyestuff as follows. When the azo-disulfide dyestuff contains a disulfide linkage,  $\text{R}-\text{S}-\text{S}-\text{R}$ , it is considered to be in its normal oxidized state. In the steamer, one molecule of the dyestuff is reduced by forming into two molecules of  $\text{R}-\text{S}-\text{Na}$ . Upon subsequent oxidation, the dyestuff is returned to its normal oxidized condition,  $\text{R}-\text{S}-\text{S}-\text{R}$ . When the azo-disulfide dyestuff is one which upon reduction and subsequent oxidation produces a disulfide group connected to aromatic nuclei, two molecules of the dyestuff ( $\text{R}-\text{S}-\text{X}$ ), wherein  $\text{X}$  may be such as a cyano or sulfonic group, are

converted by the reducing agent in the steamer to two molecules of  $R-S-Na$ , which upon subsequent oxidation are converted to  $R-S-S-R$ .

It will be understood that the above sodium atom was used for illustrative purposes and may be replaced by an equivalent cation.

Among the advantages of the above delayed action reducing agents which render them suitable for use in the method of the present invention are that they are water soluble in the printing paste, do not corrode the printing rollers, do not form into active reducing agents until heated in the steamer, neither the delayed action reducing agents nor the active reducing agents produced therefrom have an objectionable odor, the active reducing agents formed from the delayed action reducing agents are water soluble and are therefore easily removed from the fibers following oxidation, and the delayed action reducing agents are comparatively inexpensive when calculated on the basis of cost per square yard of printed material.

One of the important advantages of the method of the present invention is that a printing paste containing sulfur dye and azo-disulfide dyestuff may now be applied to the fibers. This is an important development because it provides shades and hues that cannot be obtained by use of sulfur dye or azo-disulfide dyestuff alone, and provides increased brightness of shades over that attainable by use of sulfur dye alone. Sulfur dyes are among the least expensive dyes which have generally good fastness properties, but they do not have the extraordinary brightness of color that is characteristic of the azo-disulfide dyes. By printing the azo-disulfide dyestuff and the sulfur dye together, the inherent tinctorial value of the sulfur dye and the inherent brilliance of the azo-disulfide dyestuff are obtained.

The printing paste should comprise a dyestuff selected from the group consisting of sulfur dye, azo-disulfide dyestuff, and mixture of sulfur dye and azo-disulfide dyestuff, water, thickening agent, alkali, a delayed action reducing agent selected from the group consisting of



wherein  $R_1$  and  $R_2$  are alkylene groups having 1-5 carbon atoms, a salt of said



and sodium S-sodiocarboxymethyl thiosulphate, and may additionally comprise solubilizing agent and hydroscopic agent.

The suggested composition of the printing paste, based on percent by weight of the printing paste, is given below.

The amount of dyestuff to be used in the printing paste will be determined by the depth of shade desired. Generally speaking about 1-5%, and preferably about 3% of concentrated dye will be suitable for most purposes.

The amount of delayed action reducing agent to be utilized in the printing paste will be determined by the amount of dyestuff and to some extent by the particular dye that is used, for example the sulfur blacks require somewhat more reducing agent than an equivalent amount of the other sulfur dyes. The printing paste will have 0.5-4%, and preferably about 1% of delayed action reducing agent.

The amount of alkali to be used in the printing paste will be determined by the amount of reducing agent used in the printing paste, the alkalinity of the base selected, and also by whether the salt of the di(carboxyalkyl) trithiocarbonate is formed before the di(carboxyalkyl) trithiocarbonate is incorporated into the printing paste or subsequently, more alkali being required in the printing paste when di(carboxyalkyl) trithiocar-

bonate has not been formed into a salt prior to its incorporation into the paste. About 2-12% of alkali will be suitable, and preferably about 6% when the salt of the di(carboxyalkyl) trithiocarbonate is used and preferably about 7% when the di(carboxyalkyl) trithiocarbonate is used. Any of the alkalis, such as the caustic alkalis or alkali carbonates, examples of which are  $NaOH$ ,  $KOH$ ,  $Na_2CO_3$ ,  $K_2CO_3$ , and  $NaHCO_3$  may be used.

Enough water is used to form an aqueous, alkaline dispersion of the dyestuff. The printing paste should contain a total of about 75-85%, and preferably about 80% of water.

The printing paste is thickened in the conventional manner, enough thickener being used to give the printing paste a viscosity suitable for the specific pattern desired. Any of the conventional thickeners which are compatible with free alkali may be used, such as starch, converted starches, natural gums, starch-tragacanth, water and oil emulsions, synthetic polymer thickeners, etc. Generally, about 1-7%, and preferably about 4% of thickener will be used.

A hydroscopic agent, such as diethylene glycol, monoethylene glycol, and glycerine may be advantageously used in the printing paste. About 0-4% of hydroscopic agent, and preferably about 3%, will be utilized. The hydroscopic agent is recommended, as it appears to improve color yield, but is not essential.

A solubilizing agent or assistant, such as urea, thiodiethylene glycol and glycol ethyl ether also may be advantageously used in the printing paste. About 0-4% of solubilizing agent and preferably about 3% of solubilizing agent is recommended, as it appears to improve fastness, but is not essential.

The components of the printing paste may be blended in any order, and should form a homogeneous, aqueous, alkaline dispersion. The printing paste may be prepared and applied to the fibers at room temperature, and it is recommended that the printing not be heated enough to activate the delayed action reducing agent therein prior to application to the fibers.

The above printing paste may be applied to textile fibers, such as yarns or fabrics of cotton or regenerated cellulose, singly or in blends with other fibers.

The printing paste may be applied to the fibers by any selected method, such as by a screen or by contacting the fibers with a rotating, engraved, chromium plated copper printing roller which has received the printing paste by contacting a furnish roll that rotates through and is partially immersed in a color box, a doctor blade being used to remove the paste from all except the engravings of the printing roller. It will be understood that multicolor prints and designs requiring more than one printing roller may be obtained by using additional color boxes and printing rollers.

Following application of the printing paste to the fibers, the fibers are dried sufficiently to prevent marking off of the printed areas on other areas.

Following drying, the fibers are steamed to activate the delayed action reducing agent and reduce the dyestuff. The fibers may be subjected to neutral air-free steam at  $212^{\circ}-225^{\circ} F.$  for 2-10 minutes to accomplish this result.

Following steaming, the dyestuff is oxidized. Oxidation may be accomplished by passing the fibers through a bath containing an oxidizing agent. Any of the conventional oxidizing baths used in connection with sulfur dyestuffs may be used, such as an aqueous solution of acetic acid and sodium bichromate, and aqueous solution of acetic acid and hydrogen peroxide, or an aqueous solution of ammonium persulfate. Enough oxidizing agent will be used to oxidize the dyestuff. The oxidizing agent will be customarily applied by the pad-nip method, and a bath containing 1.5 fluid oz. of glacial acetic acid and 1 oz. by weight of sodium bichromate per gallon of water is suggested. For best results, it is preferred to maintain the

xidizing bath at about 120°-140° F. Oxidation will be effected by permitting the oxidizing agent to remain in contact with the dyestuff for about 10-20 seconds.

Following oxidation, the print should be washed and dried. This may be accomplished by rinsing the print with water, soaping, rinsing with water, and drying in the conventional manner.

It will be recognized that the method of the present invention may be conducted in a continuous manner on high speed equipment positioned in tandem, such as multicolor print machine, drying cans or loop drier, rapid ager, pad boxes with nip rolls, and drying cans or oven.

The following non-limiting examples are set forth by way of illustration.

#### Example I

An aqueous, alkaline, dispersion of printing paste is made by blending together the following components in the order listed, at room temperature, all parts by weight:

| Component:                                                                  | Pounds |
|-----------------------------------------------------------------------------|--------|
| Thickener (8% aqueous solution of starch-ether)                             | 50     |
| Reducing agent di(sodiocarboxymethyl)trithiocarbonate                       | 1      |
| Hydroscopic agent (diethylene glycol)                                       | 3      |
| Solubilizing agent (urea)                                                   | 3      |
| Dye (20% aqueous dispersion Sulfur Yellow 4 solids, C.I. Part II No. 53160) | 15     |
| Water                                                                       | 22     |
| Alkali ( $\text{Na}_2\text{CO}_3$ )                                         | 6      |
| Total                                                                       | 100    |

The above printing paste is directly applied at room temperature to pre-bleached woven cotton fabric weighing 4 oz. per square yard by means of an engraved chromium plated copper roller used in conjunction with a direct type printing machine being operated at 50 yards per minute. Conventional rubber blanket and back grey are also used in conjunction with the print machine.

The fabric is dried to prevent marking off by serpentine it about 4-6 rotating, steam-heated, stainless steel, drying cans six feet in diameter and maintained at an internal steam pressure of 15-30 p.s.i.

The dyestuff is reduced by passing the fabric through a neutral ager with air-free steam at 216°-220° F. for 5 minutes.

Upon emergence from the steam ager, the dyestuff is oxidized by passing the fabric at 50 yards per minute through a three bowl padder containing 1.5 fluid oz. of glacial acetic acid and 1.0 oz. by weight of sodium bichromate per gallon of water at 130° F.

The fabric is finally rinsed, scoured and dried in the conventional manner by passing it through a pad box containing water at 150° F., through a pad box containing 0.5 oz. by weight of soap per gallon of water at 160° F., through two pad boxes containing water at 170° F., and by serpentine it about 16 rotating, cylindrical, steam-heated, stainless steel drying cans thirty inches in diameter maintained at an internal steam pressure of 50 p.s.i.

#### Example II

This example is the same as Example I above, except that viscose rayon fabric is substituted for the cotton fabric, 15 pounds of a 20% aqueous dispersion of Sulfur Blue 13 solids, C.I. Part II No. 53235, is substituted for the dye and 1 pound of di(sodiocarboxyethyl) trithiocarbonate is substituted for the delayed action reducing agent used in Example I.

#### Example III

This example is the same as Example I above, except that 15 pounds of a 20% aqueous dispersion of Sulfur Red 5 solids, C.I. Part II No. 53830, is substituted for the dye and 1 pound of di(sodiocarboxypropyl) trithiocarbonate is substituted for the delayed action reducing agent used in Example I.

#### Example IV

This example is the same as Example I above, except that 15 pounds of a 20% aqueous dispersion of Sulfur Black 11 solids, C.I. Part II No. 53290, is substituted for the dye used in Example I, and the amount of delayed action reducing agent used in Example I is increased to 2.0 pounds.

#### Example V

This example is the same as Example I, except that 15 pounds of a 20% aqueous dispersion of Sulfur Brown 10 solids, C.I. Part II No. 53055, is substituted for the dye and 1 pound of di(carboxymethyl) trithiocarbonate is substituted for the delayed action reducing agent used in Example I. Also, the amount of  $\text{Na}_2\text{CO}_3$  used in Example I is increased to 7.0 pounds.

#### Example VI

This example is the same as Example I above, except that 15 pounds of a 20% aqueous dispersion of Sulfur Green 14 solids is substituted for the dye used in Example I.

#### Example VII

This example is the same as Example I above, except that 15 pounds of a 20% aqueous dispersion of the azo-disulfide dyestuff solids formed by coupling one mole of diazotized meta-nitroaniline to one mole of 1-phenyl-3-methyl-5-pyrazolone, reducing the coupled product with sodium sulfhydrate, filtering, drying, condensing the resulting dried product with one mole of 2,4,6-trichloro-1,3,5-triazine in the presence of acetone and soda ash at 5° C., and reacting one mole of the resulting product with one-half mole of 4:4'-diaminodiphenyldisulfide at 20° C. is substituted for the dye used in Example I.

#### Example VIII

This example is the same as Example I, except that 1 pound of di(sodiocarboxyethyl) trithiocarbonate is substituted for the delayed action reducing agent utilized in Example I, and 15 pounds of a 20% aqueous dispersion of the azo-disulfide dyestuff solids formed by coupling one mole of tetrazotized 4:4'-diaminodiphenyldisulfide to two moles of 5'-chloro-3-hydroxy - 2',4' - dimethoxy-2-naphthylanilide is substituted for the dye used in Example I.

#### Example IX

This example is the same as Example I above, except that 1 pound of di(carboxymethyl) trithiocarbonate is substituted for the delayed action reducing agent used in Example I; 7 pounds of  $\text{NaHCO}_3$  is substituted for the alkali used in Example I; and 15 pounds of a 20% aqueous dispersion of the azo-disulfide dyestuff solids formed by coupling one mole of tetrazotized 2,2'-dichloro-4:4'-diaminodiphenyldisulfide to two moles of 3-hydroxy-2-naphtho-aniside is substituted for the dye used in Example I.

#### Example X

This example is the same as Example I, except that 15 pounds of a 20% aqueous dispersion of the azo-disulfide dyestuff solids formed by coupling one mole of diazotized meta-nitroaniline to one mole of 3-methyl-5-pyrazolone, reducing the resulting product with sodium sulfhydrate, filtering, drying, and condensing one mole of the dried product with one mole of 2,4,6-trichloro-1,3,5-triazine in the presence of acetone and soda ash at 5° C., and reacting one mole of the resulting product with one-half mole of 4:4'-diaminodiphenyldisulfide at 20° C. is substituted for the dye used in Example I.

#### Example XI

This example is the same as Example I, except that 15 pounds of a 20% aqueous dispersion of the dye formed by coupling one mole of diazotized 5-thiocyanato-2-amino-toluene to one mole of beta-naphthol is substituted for

the dye used in Example I, and 2 pounds of NaOH is substituted for the  $\text{Na}_2\text{CO}_3$  used in Example I.

*Example XII*

This example is the same as Example I above, except that 15 pounds of a 20% aqueous dispersion of the azo-disulfide dyestuff powder formed by diazotizing one mole of 4:4'-diaminodiphenyldisulfide, and reacting it with two moles of the sodium salt of acetoacet-ortho-aniside at pH 6.8 is substituted for the dye used in Example I.

*Example XIII*

This example is the same as Example I above except that 10 pounds of a 20% aqueous dispersion of Sulfur Red 5 solids, C.I. Part II No. 53830, and 5 pounds of a 20% aqueous dispersion of the azo-disulfide dyestuff solids formed by coupling one mole of diazotized para-nitroaniline to one mole of 1-phenyl-3-methyl-5-pyrazolone, reducing the coupled product with sodium sulfhydryl, filtering, drying, condensing the resulting dried product with one mole of 2,4,6-trichloro-1,3,5-triazine in the presence of acetone and soda ash at 5° C., and reacting one mole of the resulting product with one-half mole of 4:4'-diaminodiphenyldisulfide at 20° C. are substituted for the dye used in Example I.

*Example XIV*

This example is the same as Example I above, except that 7.5 pounds of a 20% aqueous dispersion of the azo-disulfide dyestuff solids described in Example XIII above and 7.5 pounds of a 20% aqueous dispersion of Sulfur Brown 52 solids, C.I. Part II No. 53320, are substituted for the dye used in Example I.

*Example XV*

This example is the same as Example I above, except that 6 pounds of a 20% aqueous dispersion of the azo-disulfide dyestuff solids described in Example IX above and 9 pounds of a 20% aqueous dispersion of Sulfur Red 5 solids are substituted for the dye used in Example I.

*Example XVI*

This example is the same as Example I above, except that 7 pounds of a 20% aqueous dispersion of the azo-disulfide dyestuff solids described in Example IX above and 8 pounds of a 20% aqueous dispersion of Sulfur Brown 52 solids are substituted for the dye utilized in Example I.

*Example XVII*

This example is the same as Example I above, except that 1 pound of di(carboxymethyl) trithiocarbonate is substituted for the delayed action reducing agent utilized in Example I; 2 pounds of KOH is substituted for the alkali used in Example I; and 10 pounds of a 20% aqueous dispersion of Sulfur Yellow 4 solids and 5 pounds of a 20% aqueous dispersion of the azo-disulfide dyestuff solids described in Example X above are substituted for the dye utilized in Example I.

*Example XVIII*

This example is the same as Example I above, except that 3 pounds of sodium S-sodiocarboxymethyl thiosulphate is substituted for the delayed action reducing agent utilized in Example I.

*Example XIX*

This example is the same as Example VII above, except that 3 pounds of sodium S-sodiocarboxymethyl thiosulphate is substituted for the delayed action reducing agent utilized in Example VII.

*Example XX*

This example is the same as Example XIV above, ex-

cept that 3 pounds of sodium S-sodiocarboxymethyl thiosulphate is substituted for the delayed action reducing agent utilized in Example XIV.

What we claim is:

1. A method for printing dyestuff on cellulosic textile fibers comprising the steps of applying to said fibers a printing paste comprising water, alkali, thickening agent, a dyestuff selected from the group consisting of sulfur dye, azo-disulfide dyestuff, and a mixture of sulfur dye and azo-disulfide dyestuff, and a delayed action reducing agent selected from the group consisting of



wherein  $\text{R}_1$  and  $\text{R}_2$  are alkylene groups having 1-5 carbon atoms, a salt of said



and sodium S-sodiocarboxymethyl thiosulphate; drying said fibers; steaming said fibers to activate the delayed action reducing agent and reduce the dyestuff; oxidizing the dyestuff; and washing, soaping, rinsing and drying the fibers.

2. The method according to claim 1, and further characterized in that said printing paste additionally comprises a hydroscopic agent and a solubilizing agent.

3. The method according to claim 1, and further characterized in that said salt of



is the sodium salt thereof.

4. The method according to claim 1, and further characterized in that said steaming is for 2-10 minutes at 212°-225° F. in air-free steam.

5. A printing paste comprising water, alkali, thickening agent, a dyestuff selected from the group consisting of sulfur dye, azo-disulfide dyestuff, and mixture of sulfur dye and azo-disulfide dyestuff, and a reducing agent selected from the group consisting of



wherein  $\text{R}_1$  and  $\text{R}_2$  are alkylene groups having 1-5 carbon atoms, a salt of said



and sodium S-sodiocarboxymethyl thiosulphate.

6. A printing paste as defined in claim 5, and further characterized in that it additionally comprises a hydroscopic agent and a solubilizing agent.

**References Cited**

**UNITED STATES PATENTS**

|           |         |            |       |         |
|-----------|---------|------------|-------|---------|
| 2,174,486 | 9/1939  | Chambers   | ----- | 8-37    |
| 2,663,613 | 12/1953 | Gibson     | ----- | 8-37    |
| 3,088,790 | 5/1963  | Schultheis | ----- | 8-1,213 |
| 3,097,908 | 7/1963  | Jellinek   | ----- | 8-22    |
| 3,098,064 | 7/1963  | Schultheis | ----- | 8-1,213 |

**FOREIGN PATENTS**

|         |        |          |
|---------|--------|----------|
| 590,397 | 2/1961 | Belgium. |
| 899,944 | 9/1944 | France.  |

**OTHER REFERENCES**

Derwent: Belgian Report No. 71A, pp. C1 and C2, Feb. 10, 1961.

Chem. Abstracts, vol. 49, p. 15181, 1955.

**NORMAN G. TORCHIN, Primary Examiner.**

**D. LEVY, T. J. HERBERT, Assistant Examiners.**